

Nov. 20, 1928.

1,692,725

R. S. EDMONDSON ET AL

MANUFACTURE OF ARTICLES ADAPTED TO RESIST ABRASION

Filed Feb. 9, 1926

13

Fig. 1.



Fig. 2.



Fig. 3.



Fig. 4.



Inventors  
Ralph S. Edmondson  
By Eugene Hahn  
Hogan, Deinard, Campbell & Co., attorneys.

Patented Nov. 20, 1928.

1,692,725

# UNITED STATES PATENT OFFICE.

RALPH S. EDMONDSON, OF ELIZABETH, NEW JERSEY, AND EUGENE HAHN, OF PHILADELPHIA, PENNSYLVANIA, ASSIGNORS TO AMERICAN ABRASIVE METALS COMPANY, A CORPORATION OF NEW YORK.

## MANUFACTURE OF ARTICLES ADAPTED TO RESIST ABRASION.

Application filed February 9, 1926. Serial No. 87,019.

This invention relates to the manufacture of articles adapted to resist abrasion and more particularly to pipes, troughs, chutes, etc., or liner plates therefor, used for the 5 conveyance of ashes, sand, stone or other abrading substances. According to the invention, these articles are made in the form of chilled iron castings with inserts of wear-resisting material, such as the artificial 10 oxides of aluminum and the carbids of silicon, known to the trade under various names.

In making a metal casting with wear-resisting lumps embedded therein, the practice of the art has been to attach such lumps to 15 the appropriate surface of a sand mold with adhesive material which would prevent the displacement of the lumps by the molten metal flowing into the mold. When, however, it was attempted to follow this practice 20 in connection with a "chill" mold, that is, a mold provided with a metal or cast iron chill section, the adhesive material would not adhere to the metallic surface of the mold, so that when the molten metal was poured into 25 the mold, the lumps of wear-resisting material would be dislodged from their proper positions, or float to the top, thus rendering the casting useless for the purpose for which it was intended.

These and other difficulties are obviated by the present invention, which contemplates a mold having a chill section of such character that the wear-resisting elements may be affixed thereto so securely that they will retain their places despite the disturbing influence of the flowing molten metal. This is accomplished specifically by forming recesses in the chill section at the desired places and then filling these recesses with core sand, 30 which is dried or baked therein. The lumps of wear-resisting material may then be anchored to the sand fillings by means of a suitable adhesive in the same way as in the case of the ordinary sand mold.

In the accompanying drawings, which are referred to herein and form a part hereof, are illustrated two molds prepared in accordance with certain features of the invention together with the products produced from the molds in accordance with certain other features of the invention.

Of the drawings:

Fig. 1 is a vertical longitudinal section of a mold for producing a plain or flat casting;

Fig. 2 shows in face view a portion of the 55 casting made in the mold of Fig. 1;

Fig. 3 is a transverse section of a mold for producing a curved casting; parts being broken away; and

Fig. 4 shows a perspective view of a casting 60 made in the mold of Fig. 3.

Referring to the drawings in detail, the mold of Fig. 1 comprises a drag section 6 in which is placed a chill section 7, that is a section of metal such as cast iron. This chill section 7 is formed with recesses 8, which are filled with core sand 5, baked or dried therein. To the exposed surfaces of the sand fillings are anchored lumps 9 of suitable wear-resisting material, by means of any suitable adhesive. The mold is completed by a cope section 11, having the mold recess 12, which is filled with molten iron through the pouring gate 13. The lumps of abrasive material 9, being anchored securely to the sand fillings, will retain their proper or prearranged positions during the flowing of the molten iron, so that there is produced, as shown in Fig. 2, a flat chilled iron casting 14, having embedded therein the abrasive lumps or inserts 9 which are exposed at the chilled surface 70 to protect the same from wear of abrading material passing thereover.

In Fig. 3 is illustrated a mold for making a pipe section or lining therefor and in which the mold is provided with a curved metal core or chill section 15 provided with recesses 8, sand fillings 5, and abrasive lumps 9. Fig. 4 shows a casting 16 made from this mold and having embedded therein the abrasive 80 lumps or inserts 9 exposed at the inner chilled 90 surface of the casting.

In Fig. 2 the abrasive lumps or inserts 9 are shown as arranged in transverse rows, being staggered as between the adjacent rows and 95 inclined in opposite directions, and as thus arranged, they will afford good protection to the chilled surface of the casting when used, as intended, to resist wear of abrading particles passing longitudinally of the casting. 100 It will be understood, however, that the abrasive lumps or inserts may be varied in size, shape and location to suit whatever conditions are to be met, it being evident that these conditions will differ in accordance with the 105 different uses to which the castings are to be put. The sand recesses 8 formed in the chill sections may be varied likewise, although de-

pending to some extent upon the abrasive lumps. Thus, the recesses may be round, square, or in the form of grooves, and may be run transversely, longitudinally or diagonally or otherwise, across the face of the chill section, so long as they can function in the required manner. It may be desirable, in many instances to provide a separate sand recess for each abrasive lump and of as little area as possible, so as to reduce the total area of the sand inserts to the minimum and correspondingly to increase the total area of the metallic surface of the chill section. While ordinary core sand has been found most satisfactory for filling the chill recesses, any other material possessing like properties may be used instead, the essential idea being to provide a bed of non-chill material for the anchorage of the abrasive elements in proper position within the mold.

In its broader aspects, the invention is not limited to the particular material or to the particular steps or modes of procedure herein specified by way of example, as many variations may be resorted to without departing from the main principles of the invention and without sacrificing its chief advantages.

We claim:

1. The method of casting chilled metal articles with wear-resisting inserts, which

method consists in providing a mold with a permanent chill-section formed with recesses, filling said recesses with non-chill material, anchoring to said non-chill material the wear-resisting elements, and pouring into the mold the molten metal without incorporating the non-chill material in the resultant casting.

2. The method of casting a metal article having an exposed chilled surface with wear-resisting inserts, which method consists in providing a mold with a chill section arranged to produce said chilled surface and formed with recesses, filling said recesses with non-chill material, anchoring the wear-resisting elements to said non-chill material only, and pouring into the mold the molten metal.

3. The method of casting chilled metal articles with wear-resisting inserts, which method consists in providing a mold with a chill-section formed with recesses, filling said recesses with core sand, anchoring to the sand fillings by a suitable adhesive lumps of wear-resisting material, and pouring into the mold the molten metal.

In testimony whereof, I have affixed my signature hereto.

RALPH S. EDMONDSON.

In testimony whereof, I have affixed my signature hereto.

EUGENE HAHN.